# EUROPEAN PATENT APPLICATION

(11) **EP 4 400 648 A1**
(43) Date of publication of application: **17.07.2024**
(21) Application number: 23151829.1
(22) Date of filing: 16.01.2023
(51) Int. Cl.: D21H 15/02, A24D 1/02, D21H 17/07, D21H 17/10, D21H 17/00, D21H 21/16, D21H 27/00

(54) **CIGARETTE PAPER AND A METHOD OF MANUFACTURE THEREOF**

(71) Applicant: JT International SA, 1202 Geneva (CH)
(72) Inventor: SINKINSON, Cecile, 01210 Versonnex (FR)
(74) Representative: Gill Jennings & Every LLP

(57) **Abstract**

A method of fabricating fire repellent cigarette paper for a heat-not-burn aerosol generating article is disclosed, the method (100, 300) comprising the steps of: grinding (105, 305) plant material to produce ground fibres; applying (115, 315) a treatment solution to the ground fibres, the treatment solution comprising a donor of a phosphorous group, to provide treated fibres comprising a phosphorous group; creating (135, 325) a paper pulp comprising the treated fibres and water; and inputting the paper pulp into a paper machine to form a fire repellent cigarette paper comprising 0.1% to 10% of phosphorous groups by weight of the total weight of the fire repellent cigarette paper.

## Description

### FIELD OF INVENTION

The present invention relates to wrapping papers for cigarettes, and specifically the manufacture of cigarette papers for fire repellent properties.

### BACKGROUND

Aerosol generating articles usually heat a consumable in order to generate an aerosol or vapour for user inhalation. In the past tobacco products such as conventional cigarettes have been burnt or combusted in order to create a tobacco smoke. More recently, heat-not-burn (HnB) products have been developed which do not require combustion of the tobacco consumable.

Known regulations require an entire HnB tobacco product to not be combustible. For example, a heated tobacco stick cannot be lit as a conventional cigarette. Known HnB products thus use metallised wrappers or cigarette paper that has been treated with additives in order to be non-combustible and fire-retardant. Such technologies are often non-biodegradable and can be toxic to humans or animals.

An object of the invention is to provide an effective fire repellent cigarette paper for heat-not-burn uses.

### SUMMARY OF INVENTION

According to an aspect of the invention, there is provided a method of fabricating fire repellent cigarette paper for a heat-not-burn aerosol generating article, the method comprising: grinding plant material to produce ground fibres; applying a treatment solution to the ground fibres, the treatment solution comprising a donor of a phosphorous group, to provide treated fibres comprising a phosphorous group; creating a paper pulp comprising the treated fibres and water; and inputting the paper pulp into a paper machine to form a fire repellent cigarette paper comprising 0.1% to 10% of phosphorous groups by weight of the total weight of the fire repellent cigarette paper.

In this way, a non-combustible heat-not-burn (HnB) aerosol generating article is provided with fire repellent properties and that is non-toxic and biodegradable. The improved HnB aerosol generating articles are environmentally friendly and cause significantly less pollution and environmental impact than previous methods of manufacturing heated tobacco sticks.

Known methods in the art use metallised paper or paper that has been treated with fire-retardant additives. However, such technologies typically produce polluting articles, where the metallised paper is non-biodegradable and where the treated paper is toxic to both humans and animals.

By forming cigarette paper using a paper pulp created from ground fibres treated with a treatment solution comprising a donor of a phosphorous group, the cigarette paper and the overall aerosol generating article is not combustible, complying with HnB requirements (and for example, EU or other national regulations). Providing the fire-repellent paper of the present invention thus removes the need for the undesirable metallised paper or additive-treated papers in the art.

It has been advantageously found that grinding the plant material before application of the treatment solution significantly improves the covalent bonding of the phosphorous groups to the ground fibres. When the phosphorous compound is in the treatment solution, a donor of the phosphorous group is yet to bond or graft to the tobacco fibres. After treatment (i.e. after the chemical reaction in which the donors of the phosphorous groups bond to the tobacco fibres), the phosphorous group(s) is bonded/grafted to the tobacco fibres (thus providing treated tobacco fibres). The ground plant fibres may comprise thin and lightweight "rag fibres", e.g. non-wood plant fibres, such as flax, hemp, sisal, rice straw, and/or esparto.

The fire repellent cigarette paper of the claimed invention chars instead of combusting when heated. In other words, the cigarette paper does not ignite and chars instead of burns. As such the cigarette paper acts as a fire retardant and carbon monoxide or other harmful gasses are not produced during a heating session.

Preferably, the ground fibres have an average diameter of less than 500 µm (microns). In this way, an optimal average diameter of the ground fibres ensures that a suitable amount of the phosphorous groups is bonded to the fibres to ensure an effective fire repellent cigarette paper. It has also been found that grinding the plant material to an average diameter of less than 500 µm also ensures a more homogenised fibres which improve the paper pulp and cigarette paper formed from it. The grinding may be performed by a mechanical dispersion mill and a homogenizer.

However, as will be appreciated by the skilled person, other grinding techniques can also be used. Microfibres may typically have a diameter between 60 to 400 µm, preferably between 60 to 200 µm.

Preferably the donor of the phosphorous group comprises an inositol phosphate moiety. For example, phytic acid is a compound which has an inositol phosphate moiety. Other examples include: D-myo-Inositol 1, 4, 5-triphosphate tripotassium salt, and D-myo-Inositol 1, 3, 4, 5-tetrakis(phosphate) ammonium salt. As will be appreciated by the skilled person, other phosphorus-based compounds may also be used as a donor of a phosphorous group.

It has been advantageously found that inositol phosphorus based derivatives/moieties allow multiple phosphorous groups from a same inositol phosphorus based derivative to be grafted to multiple fibres. In other words, one inositol phosphorus based derivative allows multiple covalent bonds to be bonded to a fibre. In this way, the amount of phosphorous groups / treatment solution required to get ensure effective fire repellent properties can be decreased, which improves the ease and cost of manufacture of the fire repellent cigarette paper.

It has also been found that the use of inositol phosphate derivatives in combination with rag fibres offer a highly sustainable manufacturing process for fire repellent cigarette papers.

Preferably, the fire repellent cigarette paper comprises 0.5% to 3% of phosphorous groups by weight of the total weight of the fire repellent cigarette paper. In this way, the cigarette paper provides effective fire repellent properties.

Preferably, the treatment solution comprises 0.1 to 20% of an inositol phosphate derivative by weight of the total weight of the treatment solution, preferably 3 to 10 %, and preferably wherein the inositol phosphate derivative comprises phytic acid.. In this way, the phosphorous group grafted to the cigarette paper is able to catalyse the carbonisation of the plant material fibres to form a dense and protective char layer on the fibre surface. This protective layer hinders heat transfer between adjacent and surrounding fibres, which in turn provides the fire repellent properties of the cigarette paper.

Preferably, the treatment solution comprises 1 to 40 % urea, preferably between 10 to 20 %. In this way, the treatment application step urea acts as an enabler which improves the accessibility of the phosphorous groups in the phytic acid to the individual fibres and ensure effective covalent bonding. The urea also protects the fibre material from degradation after the solution-treatment when it is heated at a later stage (e.g. to dry the pulp before it is heated or made into paper).

The application of the ground fibres with the treatment solution may be performed by soaking the fibres in the treatment solution or spraying the treatment solution onto the ground fibres.

Preferably, after applying the treatment solution to form moist treated fibres, the method comprises heating the moist fibres to form dried treated fibres and creating the pulp using the dried treated fibres.

If the ground fibres are soaked in the treatment solution, drying of the fibres is required to decrease the humidity / moisture content of the ground fibre-treatment solution mixture to approximately 5 to 20 % weight percentage (weight percentage of the total weight of the mixture). This may be done under atmospheric conditions over a time period of between five minutes to eight hours (preferably between 15 to 30 minutes) at a temperature of between 15 to 60 degrees Celsius (preferably between 40 to 60 °C (degrees Celsius)). The time periods and temperatures can be adjusted according to manufacturing requirements, as will be appreciated by the skilled person.

This drying step may not be necessary if the treatment solution is sprayed onto the ground fibres, since the moisture content of the treated fibres can be more easily controlled. However, as will be understood, the spraying step can also be used to provide a moisture content / humidity above the desired range, and a short drying step can be implemented.

Preferably, the heating comprises heating the moist fibres at 140 to 200 °C. Heating the ground fibre-treatment solution mixture ensures that the donors of the phosphorous groups in the treatment solution can effectively bond to the fibres.

Preferably, the ground fibres have an average diameter of less than 1 µm. In this way, the surface area of the fibres is further increased such that an improved covalent bonding can take place with the treatment solution and thus provide an improved fireproof cigarette paper.

Preferably, the method further comprises, prior to applying the treatment solution, using steam explosion of the plant fibres to obtain nanofibres having an average diameter of less than 500 nm (nanometres). In this way, the plant material, or lignocellulosic material, is pre-treated such that the smaller or nanofibers can be more easily obtained. Such nanofibres improve the mechanical properties of the cigarette paper (such as the resistance, filling capacity, or porosity of the paper), as well as further ensuring the grafting process (of the phosphorous groups to the fibres) is effectively performed. Fibres obtained through steam, or vapour, explosion may have a diameter between 50 to 500 nm, preferably between 50 to 100 nm.

Preferably, the method further comprises a step of refining the ground fibres. In this way, the ground fibres can be "grated" to produce fibrils. The refining step may be performed by passing the fibres through a disc refiner, such that the fibrils are formed as the fibres pass between the blades of the disc refiner.

It has been found that the fibrils enhance the bonding / grafting process (i.e. treatment with the phosphorous group treatment solution). The fibrils also provide an improved "clinging" of the fibres to each other (e.g. by electrostatic forces), which in turn improves the homogeneity of the distribution of the fibres when forming the paper sheet.

According to another aspect of the invention, there is provided a fire repellent cigarette paper, the fire repellent cigarette paper comprising 0.1% to 10% phosphorous groups by weight of the total weight of the fire repellent cigarette paper, preferably 0.5% to 3%.

Preferably, the phosphorous group comprise an inositol phosphate moiety. Examples include phytic acid (inositol hexaphosphate) or phytate as a salt, D-myo-Inositol 1, 4, 5-triphosphate tripotassium salt, and /pr D-myo-Inositol 1, 3, 4, 5-tetrakis(phosphate) ammonium salt.

Preferably, the fire repellent cigarette paper comprises ground plant fibres having an average diameter of less than 500 µm, where the phosphorous groups are covalently grafted to the ground plant fibres.

According to another aspect of the invention, there is provided an aerosol generating article for use with a heat-not-burn aerosol generating device, the aerosol generating article comprising: a tobacco component wrapped in a fire repellent cigarette paper, the fire repellent cigarette paper comprising 0.1 % to 10% of phosphorous groups by weight of the total weight of the fire repellent cigarette paper, preferably 0.5% to 3%.

The aerosol generating article may further comprise one or more downstream elements, including: a filter plug, a centre hole, a support tube (which may comprise paper), an aerosol cooling section, and/or a mouthpiece. The downstream elements may be arranged downstream of, and preferably adjacent to, the tobacco component (i.e. the aerosol generating substrate) of the aerosol generating article, such that in use aerosol generated from the tobacco component (e.g. from the application of heat) flows through the one or more downstream elements to be inhaled by a user.

Preferably, the aerosol generating article comprises a tobacco component wrapped in a fire repellent cigarette paper, the fire repellent cigarette paper comprising 0.1% to 10% of phosphorous groups by weight of the total weight of the fire repellent cigarette paper, preferably 0.5% to 3% and a downstream element including an aerosol cooling section adjacent to the downstream end of the tobacco component and a mouthpiece adjacent to the downstream end of the aerosol cooling section. Most preferably, the aerosol cooling section may be a paper tube or a section comprising a crimped polylactic acid sheet. Most preferably, the mouthpiece comprises a filter plug.

Preferably, the aerosol generating article comprises a tobacco component wrapped in a fire repellent cigarette paper, the fire repellent cigarette paper comprising 0.1% to 10% of phosphorous groups by weight of the total weight of the fire repellent cigarette paper, preferably 0.5% to 3% and a downstream element including an aerosol cooling section adjacent to the downstream end of the tobacco component, a centre hole adjacent to the downstream end of the aerosol cooling section and a mouthpiece adjacent to the downstream end of the centre hole. Most preferably, the aerosol cooling section may be a paper tube or a section comprising a crimped polylactic acid sheet. Most preferably, the mouthpiece comprises a filter plug.

Preferably, the aerosol generating article comprises a tobacco component wrapped in a fire repellent cigarette paper, the fire repellent cigarette paper comprising 0.1% to 10% of phosphorous groups by weight of the total weight of the fire repellent cigarette paper, preferably 0.5% to 3% and a downstream element including a first centre hole having a first inner diameter adjacent to the downstream end of the tobacco component, a second centre hole having a second inner diameter adjacent to the downstream end of the first centre hole and a mouthpiece adjacent to the downstream end of the second centre hole. Most preferably, the first inner diameter is smaller than the second inner diameter. The first inner diameter may be ranging from 1,5 mm (millimetre) and 4,5 mm. The second diameter may be ranging from 3,5 mm to 6,0 mm. Most preferably, the mouthpiece comprises a filter plug.

Preferably, the aerosol generating article comprises a tobacco component wrapped in a fire repellent cigarette paper, the fire repellent cigarette paper comprising 0.1% to 10% of phosphorous groups by weight of the total weight of the fire repellent cigarette paper, preferably 0.5% to 3% and a downstream element including a centre hole having an inner diameter adjacent to the downstream end of the tobacco component, an aerosol cooling section adjacent to the downstream end of the centre hole and a mouthpiece adjacent to the downstream end of the aerosol cooling section. The inner diameter of the centre hole may be ranging from 1,5 mm (millimetre) and 4,5 mm. The aerosol cooling section may be a paper tube or a section comprising a crimped polylactic acid sheet. Most preferably, the mouthpiece comprises a filter plug.

In another embodiment, the aerosol generating article according any of the previous described aerosol generating article may further comprise an upstream element. Such an upstream element may be arranged upstream of, and preferably adjacent to, the tobacco component (i.e. the aerosol generating substrate) of the aerosol generating article. The upstream element may be a filter plug made of cellulose acetate with or without a centre hole, a paper filter with or without a centre hole, or a combination thereof. Preferably, the upstream element is wrapped in the fire repellent cigarette paper together with the tobacco component.

In some other examples, it is possible that the fire repellent cigarette paper only wraps the upstream element. In such a case, the tobacco component is wrapped by commonly used cigarette paper that does not have fireproofing property.

### DESCRIPTION OF DRAWINGS

Embodiments of the present invention will now be described, by way of example only, with reference to the accompanying drawings in which:
Figure 1 shows a flowchart illustrating a method for creating a cigarette paper according to the present invention;
Figure 2 shows a flowchart illustrating another method for creating a cigarette paper according to an embodiment of the present invention;
Figures 3 to 8 show flowcharts illustrating different methods for creating a cigarette paper according to further embodiments of the present invention;
Figure 9 shows a flowchart illustrating a paper making process of the present invention;
Figure 10 shows a schematic of a fire repellent cigarette paper according to the present invention; and
Figure 11 shows a schematic of a heated tobacco stick with a fire repellent paper according to the present invention.

### DETAILED DESCRIPTION

As used herein, the terms "burn retardant" component or "fire retardant" component or "fire repellent" component or "fireproof' component or "fireproofing" component are used equally and refers to a component that reduce or even avoid the flammability of a material by either blocking the initiation of fire physically or by initiating a chemical reaction that stops or avoids the fire deployment. In the sense of the present invention, "burn retardant" or "fire retardant" or "fire repellent" or "fireproof' or "fireproofing" reduce or even prohibit the combustion of tobacco material.

As used herein, the term "a donor of a phosphorous group" refers to a chemical component that comprises at least one phosphorous atom available for covalent bonding to a substrate material, said substrate material being also called the receiver.

As used herein, the terms "inositol" or "myo-inositol" refer to a carbocyclic sugar and is the biologically important form of cyclohexane-1,2,3,4,5,6-hexol. In the context of the present invention, we specifically refer to "inositol phosphate derivative/moiety" to define an inositol component wherein at least one of the hydroxyl moieties of the inositol component is substituted with a phosphorous acid moiety. In a preferred embodiment, more than one hydroxyl moieties of the inositol component are substituted with a phosphorous acid moiety. In a most preferred embodiment, all the six hydroxyl moieties of the inositol component are substituted with a phosphorous acid moiety.

As used herein, the term "covalent bond" refers to a chemical bond that involves the sharing of electrons to form electron pairs between atoms. These electron pairs are known as shared pairs or bonding pairs. The stable balance of attractive and repulsive forces between atoms, when they share electrons, is known as covalent bonding. For many molecules, the sharing of electrons allows a stable electronic configuration.

Figure 1 shows a schematic representation of the method 100 to fabricate fire repellent cigarette paper according to the present disclosure.

Raw plant material, such as flax, hemp, sisal, rice straw, and/or esparto, is first prepared by screening and removing any contaminants or other unwanted components. These non-wood plant materials are often described as rag fibres, but it should be understood that wood-based plant material may also be used.

At step 105, the raw plant material is ground into micro and/or nano fibres of plant material by use of a mechanical dispersion mill and a homogenizer. The plant material may be ground in water to improve the dispersion of material and ensure optimal homogeneity of ground fibres. The plant material is ground into microfibres having an average diameter of between 60 to 400 µm (microns), preferably between 60 to 200 µm, and/or nanofibres having an average diameter of between 50 to 500 nm (nanometres), preferably between 50 to 100 nm. Optionally, the plant material can also be pre-treated using steam explosion to obtain nanofibres.

The plant material may be bleached, before or after the grinding step 105, to remove lignin from the plant material.

At step 110, the ground fibres are passed through a disc refiner. Disc refiners can be used to affect the structural and binding characteristics of plant or cellulose fibres. In this case, the ground fibres are abraded or grated to form fibrils on its surface which will improve the binding properties of the paper pulp mixture as well as allow the fireproofing treatment of the next step to be more effectively performed.

To fireproof the ground fibres in this specific example, the fibres are soaked in an aqueous treatment solution of a donor of phosphorous groups, in this specific example phytic acid (although other phosphorous groups may be used), and urea at step 115. The composition of the aqueous treatment solution includes:
- 0.1 to 20 % phytic acid, preferably between 3 to 10 %, and
- 1 to 40 % urea, preferably between 10 to 20 %.

The ratio of the ground fibres to the aqueous treatment solution is between 1:1 to 1:10 part material to part solution. For example, 1 gram of ground fibres to 1 ml of solution, or 1 gram of ground fibres to 10 ml of solution. Preferably, the ratio is 1 gram of ground fibres to 5 ml of aqueous treatment solution. The ground fibres are soaked in the treatment solution for a time period of between 5 to 60 minutes.

At optional step 120, the ground fibre-treatment solution mixture is filtered to remove any excess treatment solution and/or any unwanted particles from the mixture. The soaked mixture is then dried at step 125 to dry the mixture to a desired humidity level / moisture content. The drying is performed under atmospheric conditions for a period of between 5 minutes to 8 hours at a temperature of between 40 to 60 °C. The desired humidity level, or moisture content, is between 5 to 20 % as a weight percentage of the total weight of the mixture. At step 130, the partially dried mixture is then heated at a temperature of 140 to 200 °C for a duration of 2 hours for the phosphorous groups in the aqueous treatment solution to graft onto the plant fibres. A further optional washing and drying step may take place after heating step 130 to further remove any excess non-grafted treatment solution.

At step 135 water is added to the dried and heated (i.e. treated) fibres to create a pulp mixture. The pulp should have a humidity level / moisture content of approximately 95 %. Optionally, calcium carbonate can be added at this step to improve the whiteness of the paper.

The pulp of treated fibres and water is then worked through a paper machine. The paper machine includes two distinct sections: the wet section and the dry section. The wet section involves spraying and pressing, and the dry section involves drying the pressed mixture.

At step 140, the pulp mixture is continuously sprayed from a headbox 200 onto a forming wire, or forming fabric 205. The forming fabric 205 is a fine-mesh fabric from which water will be progressively sucked / removed from the overlying pulp mixture. At the end of the forming fabric 205, the pulp mixture is in the form of a sheet typically containing less than 80% water.

The sheet of pulp mixture is then transferred to the pressing or press section 210 at step 145 by a support belt, where the press section 210 is configured to extract as much water as possible from the sheet before it enters the dry section of the machine. At the end of the press section 210, the sheet typically still contains about 50% of water. Optionally the press section 210 further includes a second press for marking or embossing the paper with fine woven lines or other markings.

At step 150 the pressed sheet is transferred to the dry section, which typically involves passing the sheet through a series of heated cylinders 215 as shown in Figure 1. The cylinders 215 are typically heated with steam and the sheet is dried by conduction. As will be understood by the skilled person, different drying techniques may also be used to replace or in addition to the conduction technique of the heated cylinders 215. For example, the sheet may be dried by convection, where hot air is blown onto the sheet, and/or by radiation such as infrared to increase the temperature of the sheet.

The sheet is continuously dried, moving across the cylinders 215 until the moisture content of the paper is around 6%, where it is then further transferred to be rolled at step 155. As will be appreciated by the skilled person, the paper sheet may undergo one or more finishing treatments before it is rolled, as may be required by the paper design.

Figure 2 shows a schematic representation of another method 300 to fabricate fire repellent cigarette paper according to another specific example of the present disclosure. This second method 300 is mostly the same as the first method 100, except for the treatment of the ground fibres with the phosphorous-group treatment solution.

The grinding step 305 and the refining step 310 are the same as the grinding and refining steps 105, 100 described in reference to the first method 100 to provide ground micro and/or nano-fibres of plant material.

At step 315, the ground fibres are sprayed with the aqueous treatment solution of phytic acid (although other phosphorous groups may be used), and urea to a humidity level / moisture content of 5 to 20 %. Spraying the ground fibres allows a greater control of the moisture content of the mixture, which means that the drying step 125 in the first method 100 is not necessary in the present method 300.

After spraying, the fibres are heated at step 320 in the same way as heating step 130 in the first method at a temperature of 140 to 200 °C for a duration of 2 hours. A further optional washing and drying step may take place after heating step 320 to further remove any excess treatment solution of donor of phosphorous groups that has not grafted to the fibres. The treated fibres are then made into a pulp mixture at step 325 by added water to a moisture content of 95%, where the pulp mixture is made into paper in the same way as that described above in reference to Figure 1.

A number of the steps in the methods described above in reference to Figures 1 and 2 may be added, removed or modified as explained in the following examples. For simplicity, the different steps are set out below which may be selectively included into the different exemplary methods:

| **Step** | |
|---|---|
| 10 | grinding the plant material into ground fibres |
| 11 | refining the ground fibres |
| 20 | applying a treatment solution to the ground fibres |
| 20a | applying the treatment solution by soaking |
| 20b | applying the treatment solution by spraying |
| 21 | filtering the treated fibres |
| 22 | drying the treated fibres |
| 23 | heating the treated fibres |
| 25 | washing and filtering the treated fibres |
| 30 | creating a paper pulp |
| 40 | providing a fire repellent cigarette paper |
| 41 | spraying the paper pulp |
| 42 | pressing the paper pulp |
| 43 | drying the paper pulp |
| 44 | processing the pressed and dried paper pulp to provide the fire repellent cigarette paper |

Figure 3 shows a series of steps according to a general method 400 to manufacture fire repellent paper. Method 400 includes a grinding step 10 to grind the raw plant material into ground fibres. Grinding may include solid grinding, which involves a mechanical dispersion mill and a homogenizer to produce particles and ground fibres in the micrometre and/or nanometre scale. Step 10 may also include screening and filtering to separate out the ground fibres of the desired size (or to remove the unwanted particles / fibre sizes). Grinding step 10 may also include a pre-treatment process using steam explosion, or vapour explosion of the plant material (i.e. a lignocellulosic material) to obtain cellulose nanofibres. The pre-treatment process may also include bleaching for the removal of lignin from the plant material.

At step 20, the treatment solution comprising phosphorous group donors is applied to the ground fibres. The application of the treatment solution may be performed by soaking or spraying. As indicated by box 405, the treatment of the fibres only includes the application of the treatment solution comprising a donor of a phosphorous group. Further steps in the treatment of the ground fibres may be included to enhance the bonding of donors to the ground fibres. The composition of the treatment solution includes:
- 0.1 to 20 % phytic acid, preferably between 3 to 10 %, and
- 1 to 40 % urea, preferably between 10 to 20 %.

The ratio of the ground fibres to the aqueous treatment solution is between 1:1 to 1:10 part material to part solution.

A paper pulp is created at step 30, in which the treated fibres are mixed with water. At step 40, the paper pulp mixture is then made into a cigarette paper having fire repellent properties due to the treated fibres. The making of the paper pulp and cigarette paper may involve known process steps, as well as the steps described in the present disclosure.

Figure 4 shows another series of steps according to another method 500, similar to the general method 400 described above in reference to Figure 3. As indicated by box 505, the treating of the ground fibres to provide treated fibres comprising a phosphorous group includes applying the treatment solution at step 20, followed by a heating step 23, where the ground fibre-treatment solution mixture (also described as humid or moist treated fibres) is heated to a temperature of 140 to 200 °C, preferably for a duration of about two hours. Heating the mixture further allows the phosphorous groups in the treatment solution to effectively bond to the ground fibres. The treated fibres are mixed with water to create a paper pulp at step 30, and the paper pulp is then made into a cigarette paper having fire repellent properties at step 40. The composition of the treatment solution used at step 20 is similar to the one described for figure 3.

Figure 5A shows a series of steps according to a method 600, which is a specific example of method 500 in which the treatment of the ground fibres includes both applying a treatment solution and heating the ground fibre-treatment solution mixture to a temperature of 140 to 200 °C, as indicated by box 605. In this specific method 600, the application of the treatment solution is performed by soaking the ground fibres in the treatment solution. The soaking time of the ground fibres is between 5 to 60 minutes, preferably between 10 to 60 minutes. The treated fibres are then mixed with water to create a paper pulp at step 30, and the paper pulp is made into a cigarette paper having fire repellent properties at step 40.

Figure 5B shows another series of steps according to another method 650, which is another specific example of method 500 in which further steps are included in the treatment of the ground fibres, as indicated by box 655. After soaking the ground fibres in the treatment solution at step 20a (to apply the treatment solution to the ground fibres), the ground fibre-treatment solution mixture is filtered at step 21 to remove any excess solution and molecules from the mixture, and dried at step 22. Preferably, the mixture is dried to achieve a humidity/moisture level of 5 to 20 % (weight percentage of the total weight of the mixture) under atmospheric conditions for a duration of 5 minutes to 8 hours (ideally between 15 to 30 minutes) at a temperature between 15 to 60 °C, preferably between 40 to 60 °C. The dried mixture is then heated at a temperature of 140 to 200 °C at step 23. The treated fibres are then mixed with water to create a paper pulp at step 30, and the paper pulp is made into a fire repellent cigarette paper at step 40.

Figure 6 shows another method 700 which is another specific example of method 500 in which the treatment of the ground fibres includes both applying a treatment solution and heating the ground fibre-treatment solution mixture to a temperature of 140 to 200 °C, as indicated by box 705. In this specific method 700, the application of the treatment solution is performed by spraying the ground fibres with the treatment solution. Preferably, the ground fibres are sprayed with the treatment solution until the moist/humid treated fibres have a moisture/humidity content of 5 to 20 % (weight percentage of the total weight of the mixture). The treated fibres are then mixed with water to create a paper pulp at step 30, and the paper pulp is made into a fire repellent cigarette paper at step 40.

Figure 7 shows a method 800 similar to the general method 400 and further including a washing and filtration step after applying the treatment solution to the ground fibres. After grinding the raw plant material at step 10, the ground fibres are treated as indicated by box 805, which includes the applying of the treatment solution at step 20 and washing and filtering the treated fibres at step 25 before the treated fibres are mixed with water to form a paper pulp at step 30. Washing and filtering the treated fibres remove any excess solution and molecules. Chemically pure urea is a colourless and odourless solid that does not interfere with the colour or the mechanical properties of the final paper. The paper pulp is made into a fire repellent cigarette paper at step 40.

Figure 8 shows a method 900 in which an additional step is performed before the ground fibres are treated with the treatment solution of a donor of phosphorous groups. At step 10, the raw plant material is ground into ground fibres. At step 11, the ground fibres are refined, where the ground fibres are grated such that fibrils are formed on the surfaces of the ground fibres. This may be performed by passing the ground fibres between the blades of a disc refiner. The refined ground fibres are then soaked or sprayed with the treatment solution at step 20, mixed with water to create a paper pulp at step 30, and then the paper pulp is made into a fire repellent cigarette paper at step 40. The composition of the treatment solution used at step 20 is similar to the one described for figure 3.

Figure 9 shows a series of steps for the paper making process 1000 of step 40 previously mentioned for figures 3 to 8. The paper making process is split into a wet section 1010 and a dry section 1020. In the wet section 1010, a paper pulp made of the treated fibres and water is continuously sprayed onto a forming wire via a headbox at step 41. The forming wire is a fine-mesh fabric and water is progressively extracted from the sprayed paper pulp on the forming wire / forming fabric. As the sprayed paper pulp leaves the forming wire, the sprayed paper pulp "sheet" contains less than 80 % water, and the sheet enters the pressing or press section of the wet section 1010.

At step 42, the sheet is pressed to further extract water from the sheet of sprayed paper pulp before it enters the dry section 1020. At the end of the pressing step 42, the sheet of paper typically contains about 50% water. In some paper making processes, there can be two presses where the first one extracts water (i.e. step 42) and a second press marks the paper with fine woven lines which can control the combustion of regular / conventional cigarettes. The woven lines may control the heat distribution in heat-not-burn cigarettes. The pressed sheet then enters the dry section 1020.

In the dry section 1020, the pressed sheet is dried at step 43. The continuous sheet of paper is moved from cylinder to cylinder in the drying section 1020. There are different methods of drying the pressed sheet, including:
- Conduction, where the paper sheet is in contact with one or more heated metal cylinders. The cylinders may be heated with steam,
- Convection, where hot air is blown onto the paper sheet,
- Radiation, where infrared radiation is used to increase the temperature of the ramps in the drying section 1020.

When the paper sheet reaches a moisture content of around 6 % water it undergoes one or more finishing treatments at step 44 to provide the fire repellent cigarette paper. For example, the paper sheet may be cut into individual pieces of cigarette paper 1100 as shown in Figure 10 having predetermined dimensions (width, W and length, L), thickness and basis weight according to design and manufacturing requirements. For example, the basis weight is ranging from 20-110 gsm (g/m²), preferably ranging from 20-80 gsm, more preferably ranging from 20-65 gsm, even more preferably ranging from 25-55 gsm. For example, the thickness is ranging from 20-160 µm, preferably ranging from 20-120 µm, more preferably ranging from 20-80 µm, even more preferably ranging from 25-55 µm. As will be understood, the paper making process 1000 described above can be combined with any of the methods described in Figures 1 to 8.

Figure 11 shows an exemplary heated tobacco stick (HTS) 1200 comprising an aerosol generating substrate 1210 comprising tobacco material wrapped by a fire repellent cigarette paper according to the present disclosure. The HTS 1200 further comprises a downstream element 1220, also called the mouth end section. The mouth end 1220 may comprise multiple segments, including one or more of a filter plug, a centre hole, a support tube, an aerosol cooling section, and/or a mouthpiece. The mouth end 1220 is located downstream of, and preferably adjacent to, the tobacco component (i.e. the aerosol generating substrate 1210) of the aerosol generating article 1200, such that in use aerosol generated from the tobacco component (e.g. from the application of heat) flows through the mouth end 1220 to be inhaled by a user. In some examples, the mouth end 1220 can comprise a cooling section, such a cooling section may be a paper tube or a section comprising a crimped polylactic acid sheet. In some other example, the mouth end 1220 can comprise a first centre hole having a first inner diameter adjacent to the downstream end of the tobacco material, a second centre hole having a second inner diameter adjacent to the downstream end of the first centre hole and a mouthpiece adjacent to the downstream end of the second centre hole. In such a case, the first inner diameter is smaller than the second inner diameter. The first inner diameter may be ranging from 1,5 mm (millimetre) and 4,5 mm. The second diameter may be ranging from 3,5 mm to 6,0 mm. In another example, the mouth end 1220 can comprise a centre hole having an inner diameter adjacent to the downstream end of the tobacco component, an aerosol cooling section adjacent to the downstream end of the centre hole and a mouthpiece adjacent to the downstream end of the aerosol cooling section. The inner diameter of the centre hole may be ranging from 1,5 mm (millimetre) and 4,5 mm. The aerosol cooling section may be a paper tube or a section comprising a crimped polylactic acid sheet. The above examples should not be limiting the present invention. It will be apparent from the overall disclosure that the mouth end 1220 can combine multiple segments in a different way for providing the HTS 1200 and can also comprise an upstream element located upstream of, and preferably adjacent to, the tobacco component (i.e. the aerosol generating substrate 1210) of the aerosol generating article 1200 (not shown in Figure 11). The upstream element may be a filter plug made of cellulose acetate with or without a centre hole, a paper filter with or without a centre hole, or a combination thereof. Preferably, the upstream element is wrapped in the fire repellent cigarette paper together with the tobacco component. In some other examples, it is possible that the fire repellent cigarette paper only wraps the upstream element. In such a case, the tobacco component is wrapped by commonly used cigarette paper that does not have fireproofing property.

## Claims

1. A method of fabricating fire repellent cigarette paper for a heat-not-burn aerosol generating article, the method comprising the steps of:
grinding plant material to produce ground fibres;
applying a treatment solution to the ground fibres, the treatment solution comprising a donor of a phosphorous group, to provide treated fibres comprising a phosphorous group;
creating a paper pulp comprising the treated fibres and water; and
inputting the paper pulp into a paper machine to form a fire repellent cigarette paper comprising 0.1% to 10% of phosphorous groups by weight of the total weight of the fire repellent cigarette paper.

2. The method of claim 1, wherein the ground fibres have an average diameter of less than 500 µm.

3. The method of claims 1 or 2 wherein the fire repellent cigarette paper comprises 0.5% to 3% of the phosphorous groups by weight of the total weight of the fire repellent cigarette paper.

4. The method of claims 1, 2 or 3 wherein the donor of the phosphorous group comprises an inositol phosphate moiety.

5. The method of any preceding claim wherein the treatment solution comprises 0.1 to 20% of an inositol phosphate derivative by weight of the total weight of the treatment solution, preferably 3 to 10 %, and preferably wherein the inositol phosphate derivative comprises phytic acid..

6. The method of claim 5 wherein the treatment solution comprises 1 to 40% urea, preferably between 10 to 20%.

7. The method of any preceding claim wherein after applying the treatment solution to form moist treated fibres, the method comprises heating the moist fibres to form dried treated fibres and creating the pulp using the dried treated fibres.

8. The method of claim 7 wherein heating comprises heating the moist fibres at 140 to 200 °C.

9. The method of any preceding claim where the ground fibres have an average diameter of less than 1 µm.

10. The method of any preceding claim further comprising:
prior to applying the treatment solution, using steam explosion of the plant fibres to obtain nanofibres having an average diameter of less than 500 nm.

11. The method of any preceding claim, the method further comprising a step of refining the ground fibres.

12. Afire repellent cigarette paper, the fire repellent cigarette paper comprising 0.1% to 10% phosphorous groups by weight of the total weight of the fire repellent cigarette paper, preferably 0.5% to 3%.

13. The fire repellent cigarette paper of claim 12, wherein the phosphorous groups comprise an inositol phosphate moiety.

14. The fire repellent cigarette paper of claims 12 or 13 comprising:
ground plant fibres having an average diameter of less than 500 µm, where the phosphorous groups are covalently grafted to the ground plant fibres.

15. An aerosol generating article for use with a heat-not-burn aerosol generating device, the aerosol generating article comprising:
a tobacco component wrapped in a fire repellent cigarette paper, the fire repellent cigarette paper comprising 0.1% to 10% of phosphorous groups by weight of the total weight of the fire repellent cigarette paper, preferably 0.5% to 3%.
